

Nov. 19, 1968

D. W. SCHULZ ET AL

3,411,898

NICKEL BASE ALLOY

Filed March 25, 1966

### COMPARATIVE LARSON MILLER CURVES



INVENTORS  
DAVID W. SCHULZ  
PETER L. LANSING  
GLENN A. FRITZLEN  
BY *David W. Schulz*  
ATTORNEY

## 1

3,411,898

### NICKEL BASE ALLOY

David W. Schulz, Peter L. Lansing, and Glenn A. Fritzen, Kokomo, Ind., assignors to Union Carbide Corporation, a corporation of New York

Filed Mar. 25, 1966, Ser. No. 537,351  
2 Claims. (Cl. 75—171)

The present invention relates to nickel base alloys. More particularly the present invention relates to a nickel base alloy in wrought form characterized by improved welding properties and superior hardness, strength, and endurance properties at high temperatures.

A substantial advance in the field of nickel-base alloys over about the past decade has been the development of precipitation hardened alloys wherein the precipitate is  $\text{Ni}_3(\text{Al},\text{Ti})$ , gamma prime. The addition of particular amounts of titanium and aluminum to nickel base alloys causes the development of the aforementioned precipitate in a dispersion throughout the solid solution matrix of the alloy. Such alloys in cast form have been found to be especially useful under severe operating conditions when used as blades and vanes in gas turbine engines.

However, previously known precipitation hardened nickel-base alloys have been difficult to fabricate and, when in wrought form, are subject to serious limitations especially as regards tensile strength, durability and welding properties.

It is therefore an object of the present invention to provide a nickel base alloy which can be readily fabricated.

It is another object of the present invention to provide a nickel base alloy in wrought form characterized by improved hardness, strength, endurance and welding properties.

Other objects will be apparent from the following description and claims taken in conjunction with the drawing which shows a graph comparatively illustrating improved properties of the alloy of the present invention.

An alloy in accordance with the present invention is a precipitation-hardened nickel alloy containing

$\text{Ni}_3(\text{Al},\text{Ti})$

precipitate consisting essentially of by weight percent:

|    | Broad Range    | Preferred |
|----|----------------|-----------|
| Cr | 14 to 17       | 15.5      |
| W  | 1 to 3         | 2         |
| Fe | Up to 4.5      | 3.5       |
| C  | 0.03 to 0.13   | 0.08      |
| V  | 0.65 to 1.35   | 0.9       |
| B  | 0.003 to 0.012 | 0.007     |
| Mo | 6 to 9         | 7         |
| Al | 1.5 to 2.5     | 2         |
| Ti | 2.5 to 3.5     | 3         |
| Si | Up to 0.12     | 0.05      |
| Co | Up to 2        | <1        |
| Ni | 63 to 70       | (1)       |

<sup>1</sup> Balance.

In the present invention the rather narrow limits for the constituent materials are critical in order to obtain the improved properties hereinafter noted. For example, 14 to 17% chromium is required to provide an industrially desirable balance between ductility, strength and corrosion resistance. Chromium contents over 17%, for example tend to embrittle the alloy whereas Cr contents less than 14% tend to cause reduced strength and lessened corrosion resistance.

## 2

In the present invention it has been found that both tungsten and molybdenum must be present with the tungsten in the range of 1 to 3% and the molybdenum must be present in the range of 6 to 9%. Vanadium must be present in the alloy in the range of 0.65 to 1.35% as a carbide former and to suitably limit grain size in the alloy. Vanadium, when present in the range of 0.65 to 1.35% serves as a grain refinement agent thus enhancing ductility, strength and stability.

Titanium and aluminum must also be present in the ranges of 2.5 to 3.5% and 1.5 to 2.5% respectively in order to form the gamma prime precipitate,  $\text{Ni}_3(\text{Al},\text{Ti})$ .

With the foregoing elements present in the indicated proportions a complex matrix is formed which is very stable at elevated temperatures and has excellent strength and endurance properties.

In addition to the above mentioned constituents, boron must be present in the alloy in the range of 0.003 to 0.012% in order to improve the creep properties of the alloy as shown in Table V and also to improve the ductility of the alloy in the 1300–1350° F. range. Boron contents above 0.012% tend to depress the melting point of the alloy and embrittle it at room temperature and below.

In the present invention iron can be adventitiously present in amounts up to 4.5% maximum and preferably is not more than 3.5%. At iron contents above 4.5% restraint-weld tests have shown that iron causes a loss of strength in the alloy.

Cobalt may also be present adventitiously up to 2% and is preferably less than 1% since the presence of cobalt tends to detrimentally affect the alloy in almost all of the desired properties. Best results are obtained without cobalt and it is also important that the alloy be essentially free of manganese, zirconium, columbium and tantalum.

With regard to silicon, it has been found that this element must be limited to 0.12% maximum in order to obtain improved stress rupture properties as shown in Table I.

The composition of the alloys noted in Table I, is shown together with other pertinent alloys in Table II, and it can be seen that a very small difference in silicon content results in a very substantial difference in properties. That is to say, with reference to Table I, it can be seen that alloys 82 and 543 of this invention containing 0.06 and 0.03% silicon respectively, have much better properties than alloys 550 and 551 which contain 0.22 and 0.21% silicon and are outside the scope of the present invention.

The alloys tested and noted in Table I were in the form of 0.063" sheet and were prepared by vacuum induction melting, forging at 2100° F. to about 0.75 inch plate and hot rolling at 2100° F. to 0.063 inch sheet.

TABLE I

| Alloy     | Stress,<br>P.s.i. | Temp.,<br>° F. | Life,<br>Hours | Silicon<br>Content,<br>Percent |
|-----------|-------------------|----------------|----------------|--------------------------------|
| Alloy 550 | 75,000            | 1,350          | +2.8           | 0.22                           |
| Do        | 40,000            | 1,500          | 10.6           | 0.22                           |
| Alloy 551 | 75,000            | 1,350          | 3.0            | 0.21                           |
| Do        | 40,000            | 1,500          | 1.9            | 0.21                           |
| Alloy 82  | 75,000            | 1,350          | 116.3          | 0.06                           |
| Do        | 40,000            | 1,500          | 140.8          | 0.06                           |
| Alloy 543 | 75,000            | 1,350          | 188.7          | 0.03                           |
| Do        | 40,000            | 1,500          | 218.6          | 0.03                           |

TABLE II.—CHEMICAL ANALYSES FOR EXPERIMENTAL ALLOYS

| Alloy No. | Composition in Weight Percent |      |      |      |     |      |       |       |      |       |      |      |      |
|-----------|-------------------------------|------|------|------|-----|------|-------|-------|------|-------|------|------|------|
|           | Cr                            | W    | Fe   | C    | Si  | Co   | Ni    | Mn    | V    | B     | Mo   | Al   | T    |
| 82 1      | 15.62                         | 1.65 | 3.60 | .07  | .06 | Bal. | .01   | .96   | .005 | 7.23  | 1.90 | 2.96 |      |
| 543 1     | 15.26                         | 2.10 | 3.35 | .07  | .03 | .01  | Bal.  | .04   | .06  | .006  | 9.8  | 2.02 | 3.06 |
| 83 1      | 15.81                         | 1.67 | 3.65 | .12  | .07 | Bal. | .01   | 1.02  | .005 | 7.16  | 1.99 | 2.24 |      |
| 544       | 15.84                         | 2.15 | 3.87 | .20  | .08 | 1.08 | Bal.  | .05   | .92  | .021  | 6.60 | 2.11 | 3.02 |
| 84 1      | 15.92                         | 1.75 | 3.50 | .04  | .04 | Bal. | .01   | 1.09  | .006 | 7.28  | 1.28 | 2.66 |      |
| 546 1     | 15.55                         | 2.08 | 3.98 | .08  | .04 | .02  | Bal.  | .01   | .97  | .006  | 6.81 | 1.47 | 3.20 |
| 85 1      | 15.74                         | 1.58 | 3.50 | .03  | .08 | Bal. | ----- | 1.02  | .003 | 7.36  | 2.00 | 2.28 |      |
| 545 1     | 15.43                         | 2.19 | 3.50 | .08  | .02 | .23  | Bal.  | .01   | .91  | .009  | 7.23 | 1.55 | 2.57 |
| 2         | 15.55                         | 1.89 | 5.45 | .11  | .06 | .12  | Bal.  | .01   | .85  | .009  | 6.98 | 2.04 | 2.98 |
| 3         | 16.09                         | 1.90 | 5.45 | .12  | .05 | .12  | Bal.  | .01   | .85  | .010  | 7.10 | 2.22 | 3.10 |
| 550       | 15.13                         | 2.02 | 3.95 | .06  | .22 | .16  | Bal.  | .02   | .77  | .008  | 6.92 | 2.07 | 3.28 |
| 551       | 15.92                         | 2.13 | 3.23 | .10  | .21 | 1.10 | Bal.  | .01   | .77  | .006  | 6.98 | 1.97 | 3.28 |
| A         | 19                            | <0.5 | <1   | 0.08 | 0.3 | 11   | Bal.  | ----- | <15  | 0.005 | 10   | 1.5  | 3.2  |
| B         | 19                            | <0.5 | <1   | 0.1  | 0.2 | 13   | Bal.  | ----- | <15  | ----- | 4    | 1.2  | 2.5  |

<sup>1</sup>Alloy of this invention,.

One of the problems associated with previously known commercial alloys of the gamma prime strengthened type relates to failure of welded components in the aged condition. With these alloys characteristic cracks in the heat-affected zone and crack propagation into the parent metal are believed to result from low ductility of the material in tension. Restraint-weld tests (which involves welding a disc of the metal under test inside a "doughnut" section of the same material, using the test material for the weld, and heating to 1400° F. over 1½ hours, aging for 16 hours and air cooling) have shown, however, that alloys of this invention successfully pass this test, while previously known gamma prime strengthened commercial alloys were not uniformly satisfactory. It is believed that iron contents over about 4.5 percent in these alloys depressed the degree of hot tensile elongation in the alloys, thereby resulting in weld cracking. The following data in Table III shows that iron contents above 4.5 percent in the alloy detrimentally affects the room temperature elongation characteristics of the alloy. All specimens tested were

tion melting, forging at 2100° F. to about 0.75 inch and hot rolling at 2100° F. to 0.063 inch.

TABLE IV.—AVERAGE TENSILE PROPERTIES OF THE  
ALLOY OF THIS INVENTION

|    | Temperature, ° F. | Ultimate Strength, P.s.i. | Yield Strength, 0.2 Percent Offset, P.s.i. | Elongation, Percent |
|----|-------------------|---------------------------|--------------------------------------------|---------------------|
| 20 | Room              | 191,000                   | 143,000                                    | 21.5                |
|    | 1,000             | 176,000                   | 134,000                                    | 23.0                |
| 25 | 1,200             | 175,000                   | 132,500                                    | 14.5                |
|    | 1,300             | 173,500                   | 131,000                                    | 9.5                 |
|    | 1,400             | 160,000                   | 125,000                                    | 8.0                 |
|    | 1,500             | 142,500                   | 116,500                                    | 7.5                 |
|    | 1,600             | 117,000                   | 97,500                                     | 7.0                 |

The excellent creep-rupture properties of the present invention, which complement the aforesaid stress-rupture properties, are shown in Table V and the fabricability and welding properties of the invention are shown in Tables VI, VII and VIII. The specimens used in obtaining the data in these tables were 0.063 inch sheet prepared as above-noted and were annealed at 2050° F. for 30 minutes and water quenched but not aged.

TABLE V.—CREEP RUPTURE RESULTS FOR ALLOYS OF THIS INVENTION

| Alloy No. | Test Temperature, ° F. | Stress, P.s.i. | Life, Hours | Elongation, Percent | Time for Deformation of, Hours |        |        |        |
|-----------|------------------------|----------------|-------------|---------------------|--------------------------------|--------|--------|--------|
|           |                        |                |             |                     | 0.5%                           | 1.0%   | 2.0%   | 5.0%   |
| 84-----   | 1,350                  | 75,000         | 770.1       | 3.0                 |                                |        |        |        |
| 84-----   | 1,350                  | 75,000         | 810.7       | 2.0                 |                                |        |        |        |
| 846-----  | 1,350                  | 75,000         | 125.70      | 2.95                |                                | 48.93  | 105.10 |        |
| 846-----  | 1,350                  | 75,000         | 114.9       | 3.58                | 29.80                          | 72.50  | 99.83  |        |
| 84-----   | 1,500                  | 40,000         | 487.77      | 2.08                | 163.77                         | 375.67 | 489.67 |        |
| 546-----  | 1,500                  | 40,000         | 153.5       | 7.55                | 45.90                          | 83.30  | 112.13 | 145.80 |

in the form of 0.063 inch sheet material annealed and aged 16 hours at 1400° F.

TABLE III

| Alloy | Iron Content in Weight<br>Percent | Tensile, Elongation,<br>Percent |
|-------|-----------------------------------|---------------------------------|
| 2     | 5.45                              | 15.4                            |
| 3     | 5.45                              | 15.3                            |
| 82    | 3.60                              | 24.2                            |
| 83    | 3.65                              | 21.9                            |
| 545   | 3.50                              | 24.3                            |
| 546   | 3.93                              | 24.8                            |

The engineering test data of the "as cast" weldments of the alloy of this invention clearly show that the alloy has excellent characteristics when produced in the form of castings. Moreover, several alloys of this invention, of the compositions noted in Table II, were made in the form of castings. Each had good castability and yielded sound castings without any indication of hot-tearing which is commonly present in "gamma prime" alloys of this class.

In addition to the foregoing, the graph of FIGURE 1 shows the superiority, as regards stress rupture properties, of the present invention as compared to commercial alloys of the same type.

Table IV further illustrates the industrial importance of the present invention by showing average tensile properties for the previously noted preferred alloy of the present invention. The samples tested were in the form of 0.063 inch sheet and were prepared by vacuum induc-

TABLE VI.—BEND TEST RESULTS FOR THE ALLOY OF THIS INVENTION

| THIS INVENTION |       |                |                        |                     |
|----------------|-------|----------------|------------------------|---------------------|
| 50             | Alloy | Bend<br>Radius | Bend Angle,<br>degrees | Remarks             |
| 82             |       | 1T             | 180                    | No sign of rupture. |
| 83             |       | 1T             | 180                    | Do.                 |
| 84             |       | 1T             | 180                    | Do.                 |
| 85             |       | 1T             | 180                    | Do.                 |

TABLE VII.—OLSEN CUP TEST RESULTS FOR THE ALLOY  
OF THIS INVENTION

| Alloy   | Thickness<br>(inches) | Annealed<br>Hardness | Cup Depth<br>(inches) | Maximum<br>Load (lbs.) |
|---------|-----------------------|----------------------|-----------------------|------------------------|
| 82----- | .0671                 | Rb 95                | .491                  | 21,050                 |
| 82----- | .0671                 | Rb 96                | .530                  | 21,640                 |
| 83----- | .0637                 | Rb 93                | .480                  | 18,830                 |
| 83----- | .0637                 | Rb 95                | .486                  | 18,625                 |
| 84----- | .0668                 | Rc 39                | .338                  | 16,000                 |
| 84----- | .0668                 | Rc 41                | .365                  | 18,700                 |
| 85----- | .0592                 | Rb 80                | .582                  | 16,700                 |
| 85----- | .0592                 | Rb 79                | .559                  | 16,250                 |

TABLE VIII.—HARDNESS OF WELD TEST SPECIMENS  
FROM THE ALLOY OF THIS INVENTION

| Alloy | Weld Area Hardness | Heat Affected Zone Hardness | Hardness of Parent Metal |
|-------|--------------------|-----------------------------|--------------------------|
| 82    | Rc 26              | Rc 20-21                    | Rb 94-99                 |
| 83    | Rb 90-96           | Rc 94-96                    | Rb 92-94                 |
| 84    | Rc 27              | Rc 28-32                    | Rc 33-36                 |
| 75 85 | Rb 85-86           | Rb 81-82                    | Rb 78-79                 |

The bend tests of Table VI were performed using specimens 6 x  $\frac{1}{16}$ " strips from 0.063" hot rolled sheet and the results show that the alloys of the present invention were capable of being bent 180° around a radius equal to the thickness of the specimen. There was no sign of rupture in the specimen after the test. The results of the standard Olsen Cup test shown in Table VII illustrate the ability of the alloy of the present invention to be easily and successfully shaped and formed into useful articles.

The weld tests of Table VIII involved clamping two specimens in a copper jig positioned for butt welding and Heliarc welding using 9-95 amperes at 12-14 volts with 30 c.f.h. argon cover gas and filler wire formed of the base alloy. These tests show that alloy of the present invention is highly suitable for welded articles.

The following schedule describes an effective heat treatment for the alloy of the present invention and except where otherwise stated all data set forth in the specification were obtained from specimens that were treated according to the schedule:

- I. Anneal for 30 minutes at 2050° F.
- II. Water quench
- III. Age 16 hours at 1400° F.
- IV. Air cool

What is claimed is:

1. A nickel base alloy consisting essentially of by weight about

|                | Percent      | 30 |
|----------------|--------------|----|
| Chromium ----- | 14 to 17     |    |
| Tungsten ----- | 1 to 3       |    |
| Iron -----     | up to 4.5    |    |
| Carbon -----   | 0.03 to 0.13 |    |

|    |                                                                          |                |
|----|--------------------------------------------------------------------------|----------------|
| 5  | Vanadium -----                                                           | 0.65 to 1.35   |
|    | Boron -----                                                              | 0.003 to 0.012 |
|    | Molybdenum -----                                                         | 6 to 9         |
| 10 | Aluminum -----                                                           | 1.5 to 2.5     |
|    | Titanium -----                                                           | 2.5 to 3.5     |
|    | Silicon -----                                                            | up to 0.12     |
|    | Cobalt -----                                                             | up to 2        |
|    | Nickel -----                                                             | balance        |
| 15 | 2. An alloy in accordance with claim 1 having the following composition: | Percent        |
|    | Chromium -----                                                           | 15.5           |
|    | Tungsten -----                                                           | 2              |
|    | Iron -----                                                               | up to 3.5      |
|    | Carbon -----                                                             | 0.08           |
|    | Vanadium -----                                                           | 0.9            |
|    | Boron -----                                                              | 0.007          |
|    | Molybdenum -----                                                         | 7              |
| 20 | Aluminum -----                                                           | 2              |
|    | Titanium -----                                                           | 3              |
|    | Silicon -----                                                            | up to 0.05     |
|    | Cobalt -----                                                             | less than 1    |
|    | Nickel -----                                                             | balance        |

25

#### References Cited

##### UNITED STATES PATENTS

|           |         |                       |        |
|-----------|---------|-----------------------|--------|
| 3,061,426 | 10/1962 | Bieber -----          | 75-171 |
| 3,183,084 | 5/1965  | Heydt et al. -----    | 75-171 |
| 3,343,950 | 9/1967  | Richards et al. ----- | 75-171 |
| 3,368,888 | 2/1968  | Winter -----          | 75-171 |

RICHARD O. DEAN, Primary Examiner.